

## UNITED STATES PATENT OFFICE.

RICHARD R. WALTER, OF DUSSELDORF, GERMANY.

## PROCESS OF DESULPHURIZING MOLTEN METAL AND BRIQUETTES USED THEREFOR.

No Drawing. Application filed March 16, 1922, Serial No. 544,332, and in Germany April 8, 1921.

My invention relates to improvements in the process of desulphurizing metal, and more particularly molten metal contained in ladles, by means of compounds of alkali metals or alkaline earth metals, or mixtures thereof, or other desulphurizing media. In the process now in use the said media are brought on the surface of the metal in the natural or pulverulent or crystalline state, and I have found that when thus applying the said media to the metal the media are thrown more or less into the surrounding air by the gases generated from the liquid metal and the whirls of air produced on the surface of the metal, which results in a loss of desulphurizing media and injury to the attendants. The object of the improvements is to obviate this objectionable feature of the process now in use, and with this object in view I form the said pulverulent or crystalline matter into pieces of granular form, and throw the said pieces on the surface of the metal. I have found that when thus using the desulphurizing media they melt on the surface of the metal without any loss. Furthermore the media melt with greater speed by reason of their more coherent state and their increased heat conducting capacity.

In the practice of my invention I use any known or preferred methods for thus forming the desulphurizing media into pieces. One method consists in melting the media and casting the same in suitable moulds. Another method consists in making blocks of suitable size by means of suitable binding media such for example as hydraulic cement or lime, and a third method consists in forming the media into bricks by means of a suitable binding medium such as tar and under high pressure.

I claim:

1. The process of desulphurizing molten metal, which consists in introducing an alkali metal compound as a cast piece of predetermined size in a quantity of molten metal.
2. The process of desulphurizing molten metal, which consists in associating with an industrially conventional quantity of molten metal a single premelted and solidified portion of an alkali metal compound.
3. The process of desulphurizing molten metal, which consists in introducing in a quantity of molten metal a mixture of an alkali metal compound and an alkaline earth metal compound as a cast piece of predetermined size.
4. The process of desulphurizing molten metal, which consists in associating with an industrially conventional quantity of molten metal a single premelted and solidified lump mixture of an alkali metal compound and of an alkaline earth metal compound.
5. The process of desulphurizing molten metal, which consists in associating with a given quantity of the molten metal, a unitary premelted mass of a dry desulphurizing compound of alkali character and of predetermined size in proportion to the quantity of molten metal.
6. The herein described process of desulphurizing molten metal, which consists in associating with the molten metal, a desulphurizing media in the form of a piece sufficiently heavy to prevent its being thrown up from the surface of the molten metal by the gases generated at the surface thereof and sufficiently dry for prevention of an explosion.
7. As a new article of manufacture a desulphurizing briquette composed of a completely fused compound of alkali character.

In testimony whereof I affix my signature.  
RICHARD WALTER.